

## 1

3,393,040

**SILVER HALIDE PHOTOGRAPHIC ELEMENTS  
CONTAINING SULFONIC ACID SUBSTITUTED  
AROYLACETARYLIDE COUPLERS**

Marcel Hendrik Verbrugghe, Wilrijk-Antwerp, Arthur Henri De Cat, Mortsel-Antwerp, and Valère Frans Danckaert, Boechout, Belgium, assignors to Gevaert Photo-Producten N.V., Mortsel, Belgium, a company of Belgium  
No Drawing. Filed July 8, 1964, Ser. No. 381,238  
Claims priority, application Belgium, July 9, 1963,  
42,771, Patent 634,669  
8 Claims. (Cl. 96—74)

This invention relates to the production of photographic color images, to the color couplers for yellow used therein and to photographic material containing such color couplers.

It is known that for the production of a photographic color image in a light-sensitive silver halide emulsion layer, the exposed silver halide is developed to a silver image with an aromatic primary amino compound in the presence of a color coupler by means of which, by reaction with the oxidized developing substance, a dye-stuff is formed on the areas corresponding with the silver image.

In the subtractive three-color photography is mostly used a light-sensitive photographic color material containing a red-sensitized, a green-sensitized and a blue-sensitive silver halide emulsion layer wherein by the use of appropriate color couplers in the color development a cyan, magenta and yellow dyestuff image respectively is formed.

It is known that color couplers have to meet different requirements according to the way wherein the color material is prepared and the object for which it is used.

For producing a usable photographic multilayer color image containing the color couplers for the different color part images in the differently sensitized silver halide emulsion layers, the color couplers shall be present in diffusion-fast form in the hydrophilic silver halide emulsion layer. This can, be realized e.g. by using a color coupler which is sufficiently water-soluble and which is provided with a sufficiently extensive organic radical in order to prevent diffusion of the color coupler into the hydrophilic silver halide emulsion layer, or by the use of a lipophilic color coupler which dissolved in an organic solvent is dispersed in the silver halide emulsion layer.

For the production of color images, more particularly of positive color images, e.g. on a paper support, it is of importance to dispose of color couplers which on color development form dyestuffs which are very stable to light, humidity and heat.

Now has been found a class of color couplers for yellow of the ketomethylene type, more especially of the aroylacetylarylide type the representatives of which in the color development form with an aromatic primary amino developing substance dyestuffs which possess a very good light, humidity- and heat-stability.

These ketomethylene color couplers of the aroylacetylarylide type are characterized by the presence of at least one sulfonic acid group in the aroyl part of the molecule and by the presence of at least one sulfonic acid group in the arylide part of the molecule.

Thus one or more sulfonic acid groups may directly be implanted on the aromatic nucleus of the aroyl group and in the same molecule one or more sulfonic acid groups may directly be implanted on the aromatic nucleus of the arylide group.

Thus, also at least one of the aromatic nuclei of the aroyl- and of the arylide group can be bound by means of a bivalent radical with an aromatic nucleus substituted by at least one sulfonic acid group.

Examples of color couplers for yellow according to the

## 2

present invention wherein at least one sulfonic acid group is implanted directly on the aromatic nucleus of the aroyl group and at least one sulfonic acid group directly on the aromatic nucleus of the arylide group, are represented by the following general formula:



wherein:

R<sub>1</sub> represents a sulfonic acid group or salt form thereof,  
R<sub>2</sub> represents a hydrogen atom, a substituent such as for instance a halogen atom, a sulfonic acid group or a salt form thereof, or a diffusion-fast making group such as e.g. an organic group containing an acyclic aliphatic radical with 5 to 20 carbon atoms such as e.g. a n-hexadecyloxy group,

R<sub>3</sub> represents a sulfonic acid group or a salt form thereof,  
R<sub>4</sub> represents a hydrogen atom, a substituent such as e.g. a halogen atom, a sulfonic acid group or a salt form thereof or a diffusion-fast making group such as e.g. an organic group containing an acyclic aliphatic radical with 5 to 20 carbon atoms such as, e.g. an n-hexadecyloxy group of an n-hexadecylmercapto group, and  
R<sub>3</sub> and R<sub>4</sub> together can represent the necessary atoms for forming a sulfonyl substituted aromatic system which may be further substituted.

Examples of color couplers for yellow according to the present invention, wherein at least one sulfonic acid group in the aroyl part of the molecule is bound on an aromatic nucleus which is linked with the aromatic nucleus of the aroyl group by a bivalent radical correspond to the following general formula:



wherein:

R<sub>2</sub>, R<sub>3</sub> and R<sub>4</sub> have the same significance as given in Formula I,

R'<sub>1</sub> represents a sulfonated aromatic radical either further substituted or not, such as e.g. a sulfonated phenyl group, and

Y represents a bivalent radical such as e.g. a —CONH— group, a —SO<sub>2</sub>NH— group or a —NHCONH— group.

Examples of color couplers for yellow according to the present invention, wherein at least one sulfonic acid group in the arylide part of the molecule is bound on an aromatic nucleus, which is linked by a bivalent radical with the aromatic nucleus of the arylide group, correspond to the following general formula:



wherein:

R<sub>1</sub>, R<sub>2</sub> and R<sub>4</sub> have the same significance as given in Formula I,

R''<sub>1</sub> represents a sulfonated aromatic radical either further substituted or not, such as e.g. a sulfonated phenyl group, and

Y<sub>1</sub> represents a bivalent radical such as e.g. a —CONH— group or a —SO<sub>2</sub>NH— group.

Examples of color couplers for yellow according to the

the present invention, wherein at least one sulfonic acid group in the aroyl part of the molecule is present on an aromatic nucleus linked by a bivalent radical with the aromatic nucleus of the aroyl group, and wherein at least one sulfonic acid group in the arylide part of the molecule is present on an aromatic nucleus linked by a bivalent radical with the aromatic nucleus of the arylide group, correspond to the following general formula:



wherein:

$\text{R}_2$  and  $\text{R}'_4$  have the same significance as given in Formula I,  
 $\text{Y}$  and  $\text{R}'_1$  have the same significance as given in Formula II, and  
 $\text{Y}'_1$  and  $\text{R}''_1$  have the same significance as given in Formula III.

The following reaction scheme illustrates the preparation of color couplers for yellow according to the general Formula I:



Herein  $\text{R}_2$  or  $\text{R}_3$  can contain a diffusion-fast making group.

Hereinafter follows a list of structural formulae of color couplers for yellow according to the present invention:



The following description illustrates more in detail the above given reaction scheme and the preparation of intermediate products of color couplers for yellow according to the present invention.

### 1. PREPARATION OF ACID CHLORIDES USED IN SYNTHESIS OF THE $\beta$ -KETOESTER DERIVATIVES

The preparation of these acid chlorides is performed as described in the Belgian patent specification 634,665 filed July 9, 1963.

### 2. PREPARATION OF THE $\beta$ -KETOESTER DERIVATIVES

The preparation of the fluorosulfonyl-substituted  $\beta$ -ketoester derivatives has also been described in said Belgian patent specification.

### 3. PREPARATION OF FLUOROSULFONYL SUBSTITUTED BENZOYL ACETANILIDES AND ALKALINE HYDROLYSIS TO SULFONIC ACID DERIVATIVES

(a) Amino derivatives used (mentioned in Table 1)

2-n-hexadecyloxy-5-fluorosulfonylaniline (Belgian patent specification 590,934)

2-n-hexadecylthio-5-fluorosulfonylaniline (Belgian patent specification 587,525)

3-fluorosulfonyl-4-n-hexadecyloxyaniline.

First p-n-hexadecyloxynitrobenzene is sulfonated at about 60° C. with sulfuric anhydride in tetrachloroethane. The reaction mixture is left for cooling overnight, the precipitate formed is separated and washed with hexane. The crude sulfonic acid derivative is then converted by neutralization with 2 N sodium hydroxide into the sodium salt. After salting out with aqueous sodium chloride, a white to greyish amorphous product is obtained which is recrystallized from acetonitrile. The 3-sulfo-4-n-hexadecyloxynitrobenzene is obtained in the form of a white crystalline product. Melting point: above 250° C.

This nitrobenzene derivative is converted into the corresponding sulfochloride by treatment with thionylchloride at boiling temperature in the presence of dimethylformamide. After evaporating the excess of thionylchloride and treating with a mixture of benzene and hexane, the 3-chlorosulfonyl-4-hexadecyloxynitrobenzene is obtained as a light-brown to white product. Melting point: 56° C.

Now this compound is allowed to react for 1 hour with potassium fluoride in acetic acid at reflux temperature. After pouring out the reaction mixture into water, separating the precipitate formed and recrystallizing from ethanol, the white crystalline 3-fluorosulfonyl-4-n-hexadecyloxynitrobenzene is obtained. Melting point: 72° C.

This nitro compound is now reduced with iron and hydrochloric acid in ethanol medium at reflux temperature. After the reduction, the reaction mixture is filtered and the amine is separated as hydrochloride. This hydrochloride is suspended in methylene chloride and treated with aqueous sodium dicarbonate. Hereby the amine is set free. After separating the organic layer and evaporating off the solvent, the crude product is recrystallized from acetonitrile. White needle-shaped 3-fluorosulfonyl-4-n-hexadecyloxylaniline crystals are obtained. Melting point: 68° C.

3 - fluorosulfonyl - 4 - n - hexadecylmercaptoaniline (Belgian patent specification 587,525).

3-fluorosulfonylaniline (British patent specification 308,276).

2-chloro-5-fluorosulfonylaniline (British patent specification 808,276).

(b) Preparation of the corresponding benzoylacetanilides

GENERAL METHOD

0.1 mol of amino derivative, 0.1 mol of  $\beta$ -ketoester derivative and 0.2 g. of anhydrous sodium acetate are brought into 100 ccs. of anhydrous xylene. The reaction mixture is heated up to reflux temperature, whereafter a mixture of xylene and the ethanol formed is slowly distilled off until the temperature has risen to 138° C. which lasts about 1 hour.

Thereafter, the remaining xylene is distilled off under reduced pressure. 200 ccs. of hexane are added to the residue. The precipitate formed is filtered off and recrystallized from a suitable solvent.

In Table 1 (col. 3-4) are given the results of condensations of amines with  $\beta$ -ketoesters.

(c) Alkaline hydrolysis to sulfonic acid derivatives of fluorosulfonyl substituted benzoylacetanilides

GENERAL METHOD

0.1 mol of sulfonylfluoride is heated with 400 ccs. of acetone to boiling temperature. Whilst stirring, 100 ccs. of 5 N sodium hydroxide (or potassium hydroxide) are slowly added. An exothermic reaction takes place. The reaction mixture is heated for 30 minutes at room temperature, whilst stirring, and afterwards acidified with acetic acid, whereafter it is cooled down to room temperature. The precipitate formed is washed with water and recrystallized from a suitable solvent.

In Table 1 (col. 5 and 6) are given the results of these alkaline hydrolyses. Column 7 refers to the above-mentioned structural formulae of color couplers for yellow according to the present invention.

TABLE I

| Amino derivative used                      | $\beta$ -Ketoester derivative used                                                  | Substituted benzoylacetanilide |                     | Sulfonic acid derivative |                         | Number of the structural formula of the color coupler |
|--------------------------------------------|-------------------------------------------------------------------------------------|--------------------------------|---------------------|--------------------------|-------------------------|-------------------------------------------------------|
|                                            |                                                                                     | Recrystallizing agent          | Melting point (°C.) | Recrystallizing agent    | Kind of the alkali salt |                                                       |
| 2-hexadecyloxy-5-fluorosulfonylaniline.    |  | Ethanol.....                   | 115-116.....        | Methanol/water.....      | Na-salt.....            | 1                                                     |
| Do.....                                    | Same as above.....                                                                  | Methanol.....                  | 87.....             | do.....                  | K-salt.....             | 2                                                     |
| Do.....                                    |  | Isopropanol.....               | 103.....            | Isopropanol/water.       | Na-salt.....            | 3                                                     |
| 2-n-hexadecylthio-5-fluorosulfonylaniline. |  | Benzene.....                   | 120.....            | Ethanol/water.....       | do.....                 | 4                                                     |
| Do.....                                    | Same as above.....                                                                  | Ethanol.....                   | 73.....             | Methanol/water.....      | Na-salt.....            | 5                                                     |
| 4-n-hexadecyloxy-5-fluorosulfonylaniline.  | do.....                                                                             | Isopropanol.....               | 142.....            | Isopropanol/water.       | K-salt.....             | 6                                                     |
| 4-n-hexadecylthio-5-fluorosulfonylaniline. | do.....                                                                             | Ethanol.....                   | 123.....            | Ethanol/water.....       | do.....                 | 7                                                     |
| 3-fluorosulfonylaniline.....               |  | do.....                        | 115.....            | do.....                  | do.....                 | 8                                                     |
| 2-chloro-5-fluorosulfonylaniline.          | Same as above.....                                                                  | Aceton/methanol.....           | 150.....            | Isopropanol/water.       | do.....                 | 9                                                     |

As specific example of a color coupler for yellow according to the present invention, wherein a sulfonic acid group in the aryl part of the molecule is bound on an aromatic nucleus which is linked by a bivalent radical with the aromatic nucleus of the aryl group, is mentioned a color coupler having the following structural formula:

11.



The following reaction scheme illustrates the synthesis of this color coupler:

(a')



5

general method described under 3(b). One starts from 41.5 g. of 2-n-hexadecyloxy-5-fluorosulfonylaniline (prepared as described in the Belgian patent specification 590,934) and 23.7 g. of 4-nitrobenzoyl acetic acid ethyl ester, and after recrystallization from benzene the yellow crystalline nitro derivative is obtained. Melting point: 104° C.

## SYNTHESIS STEP b'

This obtained nitro derivative is dissolved in ethylene glycol monomethylether and converted into the corresponding amine by hydrogenation in the presence of Raney-nickel as catalyst. The reduction is carried out under 35 kg./sq.cm hydrogen pressure and at 80° C. After reaction of the calculated amount of hydrogen, the catalyst is filtered off. In the filtrate is formed a precipitate which is separated and recrystallized from dichloroethane. The  $\alpha$ -(4'-aminobenzoyl)-2-n-hexadecyloxy-5-fluorosulfonylacetanilide is obtained in the form of a white crystalline product. Melting point: 143° C.

20

## (b) 3-fluorosulfonylbenzoylchloride

(Prepared as described in the Belgian patent specification 634,665 filed July 9, 1963.)

## 2. REACTION OF THE AMINE DERIVATIVE WITH 3-FLUOROSULFONYLBENZOYLCHLORIDE

## SYNTHESIS STEP c'

The synthesis is analogous to that described in the above-mentioned Belgian patent specification. One starts from 12.12 g. of amine derivative and an equivalent amount of 3-fluorosulfonylbenzoyl chloride. After recrystallization from dichloroethane, a white crystalline product is obtained. Melting point: 186-187° C.

## 3. ALKALINE HYDROLYSIS TO SULFONIC ACID DERIVATIVE

## SYNTHESIS STEP d'

The alkaline hydrolysis of the former sulfonylfluoride derivative is carried out analogously as indicated for the compounds mentioned under the general Formula I. After recrystallization from a mixture of ethanol and

(b')



25

(c')



35

(d')



40

## 1. SYNTHESIS OF THE STARTING PRODUCTS

(a)  $\alpha$ -(4'-aminobenzoyl)-2-n-hexadecyloxy-5-fluorosulfonylacetanilide



## SYNTHESIS STEP a'

The synthesis of the  $\alpha$ -(4'-nitrobenzoyl)-2-n-hexadecyloxy-5-fluorosulfonylacetanilide is analogous to the

12.



60



65

13.



70

75

75

The preparation of these color couplers is carried out analogously to that shown in the last mentioned reaction scheme. Only the structure of the amine differs.

### 1. SYNTHESIS OF THE AMINE DERIVATIVES

#### (a) 3-(2'-n-hexadecyloxy-5'-fluorosulfonylphenylaminofulfonyl)-aniline



First, the 3-(2'-n-hexadecyloxy-5'-fluorosulfonylphenylaminofulfonyl)-nitrobenzene is synthesized by refluxing for 30 minutes at boiling temperature an equivalent amount of m-nitrobenzene sulfochloride on 2-n-hexadecyloxy-5-fluorosulfonylaniline (Belgian patent specification 590,934). Next, the solvent is distilled off and the oil residue is treated with methanol. After washing the obtained precipitate with water and recrystallizing from methanol, the nitrobenzene derivative is obtained as a white finely granular product. Melting point: 99° C.

This nitro derivative is dissolved in ethanol and converted into the corresponding amine by hydrogenation in the presence of Raney-nickel as catalyst. The reduc-

First, the 2-n-hexadecyloxy-5-(3'-fluorosulfonylphenylaminosulfonyl)-nitrobenzene is prepared in an analogous way as given here-above under (a), starting from 3-fluorosulfonylaniline and 2-n-hexadecyloxy-5-chlorosulfonylnitrobenzene (Belgian patent specification 590,934). After recrystallization from ethanol, white crystals of the nitro derivative are obtained. Melting point: 112° C.

This nitro derivative is reduced in analogous way as indicated under (a). The 2-n-hexadecyloxy-5-(3'-fluorosulfonylphenylaminosulfonyl)-aniline is obtained as a white crystalline product. Melting point: 103° C.

### 2. PREPARATION OF THE SUBSTITUTED BENZOYLACETANILIDES

This preparation is carried out in a way analogous to that of the substituted benzylacetanilides, used in the preparation of color couplers according to the general Formula I. The results of this synthesis are given in the comparative Table 2 (col. 3 and 4).

### 3. ALKALINE HYDROLYSIS OF THE FLUOROSULFONYL SUBSTITUTED BENZOYLACETANILIDES TO SULFONIC ACID DERIVATIVES

This hydrolysis is likewise carried out in a way analogous to that of the fluorosulfonyl substituted benzylacetanilides mentioned for the preparation of color couplers according to the general Formula I.

The results of this alkaline hydrolysis are given in Table 2 (cols. 4 and 5).

TABLE 2

| Amine derivative used | $\beta$ -Ketoester used | Substituted benzylacetanilide |                      | Sulfonic acid derivative (Na-salt) |                                                       |
|-----------------------|-------------------------|-------------------------------|----------------------|------------------------------------|-------------------------------------------------------|
|                       |                         | Recrystallizing agent         | Melting point (° C.) | Recrystallizing agent              | Number of the structural formula of the color coupler |
|                       |                         | Isopropylether.....           | 120                  | Methanol/water.....                | 12                                                    |
|                       | Same as above.....      | Isopropanol.....              | 120                  | do.....                            | 13                                                    |

tion is carried out at 105 kg./sq. cm. hydrogen pressure and at 80° C. After recrystallization from methanol, the 3-(2'-n-hexadecyloxy - 5' - fluorosulfonylphenylaminosulfonyl)-aniline is obtained as a white crystalline product. Melting point: 99.5° C.

#### (b) 2-n-hexadecyloxy-5-(3'-fluorosulfonylphenylaminosulfonyl)-aniline



Attention is drawn to the fact that the color couplers need not necessarily first be separated as sulfonic acid derivatives before their addition to the silver halide emulsion, but that the sulfonic acid derivatives formed in situ from the sulfonyl fluoride derivatives, by reacting the latter with alkali, can be added as such to the emulsion. For that purpose, preferably 1 mol of sulfonylfluoride derivative is dissolved in an aqueous solution of 3 mol of sodium hydroxide and the resulting clear solution, after adjusting the pH to agree with the pH of the emulsion applied, is added to the silver halide emulsion as a 5 or 10% aqueous solution.

During the preparation of the light-sensitive color material, the non-migratory color couplers for yellow according to the above given general formulae are, preferably immediately before coating, homogeneously mixed in dissolved form with the light-sensitive silver halide

emulsion. They may also be added to the composition of a water-permeable non-light-sensitive layer being in direct contact with the light-sensitive silver halide emulsion layer or they can be incorporated into a non-light-sensitive layer which is separated from the light-sensitive layer by a water-permeable non-light-sensitive layer. The silver halide emulsion contains the usual colloids such as e.g. gelatin, polyvinylalcohol, collodion or other suitable natural or synthetic colloids. The photographic emulsion can further contain usual ingredients such as hardeners, chemical sensitizers, optical sensitizers, plasticizers, development activators, stabilizers and wetting agents.

The color couplers for yellow according to the above given general formulae are usually added to a blue-sensitive silver halide emulsion. According to the most conventionally applied procedure this silver halide emulsion is coated as first color coupler containing layer of a photographic multilayer color material. Such photographic multilayer color material usually consists successively of a support, a red-sensitized silver halide emulsion layer with color coupler for cyan, a green-sensitized silver halide emulsion layer with color coupler for magenta and a blue-sensitive silver halide emulsion layer with color coupler for yellow. The support for this multilayer material can consist of paper, glass, cellulose nitrate, a cellulose ester such as cellulose triacetate, polyester, polystyrene or any other synthetic or natural resin.

Between the silver halide emulsion layer which contains a color coupler for yellow and the green-sensitive

5

10

15

20

25

According to the invention, an exposed silver halide emulsion layer is developed with an aromatic primary amino developing substance in the presence of the color couplers for yellow according to the present invention for obtaining photographic color images.

All color developing substances capable of forming azomethine dyestuffs can be utilized as developers. The color couplers for yellow according to the present invention form on color development with aromatic primary amines, such as e.g. N-diethyl-p-phenylenediamine, yellow dyestuffs which excel by their favorable light-absorption in the blue-region of the spectrum and their poor absorption in the other regions. Further, these dyestuffs possess besides a good heat and humidity stability also a good light stability which is shown by comparative tests the description and results follow hereinafter.

The resistance to humidity and heat of the dyestuffs to be examined is determined from the decrease in density of a developed wedge print after having stored, said wedge print for some determined time (e.g. 7 days) at some determined temperature (e.g. 38° C.) and relative humidity (e.g. 95%), while protected from light.

The following table gives a clear showing of the humidity and heat stability of dyestuffs formed by the color development by reaction of the oxidation product of N-diethyl-p-phenylenediamine formed thereby with a color coupler according to the present invention and of the known color couplers respectively mentioned in the British patent specifications 808,276 and 783,887.

| Formula of the color coupler                                                         | Maximum density at the beginning of the test | Maximum density after 7 days of storing at 38° C. at 95% relat. humidity | Percent decrease in max. density |
|--------------------------------------------------------------------------------------|----------------------------------------------|--------------------------------------------------------------------------|----------------------------------|
|   | 1.20                                         | 1.13                                                                     | 6                                |
|  | 1.20                                         | 1.16                                                                     | 3                                |
|  | 1.20                                         | 0.97                                                                     | 20                               |
| (color coupler for yellow according to British patent specification 808,276)         |                                              |                                                                          |                                  |
|  | 1.20                                         | 0.86                                                                     | 29                               |
| (color coupler for yellow according to British patent specification 783,887)         |                                              |                                                                          |                                  |

silver halide emulsion layer there is usually a yellow filter layer which in most cases contains colloidal silver dispersed in gelatin. The sulfonylfluoride derivatives can be used as color couplers for yellow in the so-called droplet emulsions (cf. United States patent specification 2,304,-940.

70

75

The resistance to light of the dyestuffs formed on development with N-diethyl-p-phenylenediamine and which are to be examined is determined from the decrease in density of a developed wedge print on exposing said wedge print for some determined time (e.g. 16 hours) to the light of a "Xenon-Arc-Fade-Ometer" (daylight spectrum).

The following table gives a clear showing of the light stability of a dyestuff formed on development by reaction of the oxidation product of N-diethyl-p-phenylenediamine formed thereby with a color coupler according to the present invention and known color couplers for yellow.

substituted with a bivalent radical linked to a sulphonic acid-substituted phenyl group, said bivalent radical being a member of the group consisting of a —CONH— group, a —SO<sub>2</sub>NH— group, and a —NHCONH— group.

5 3. A photographic multi-layer color material contain-

| Formula of the color coupler                                                 | Maximum density at the beginning of the test | Maximum density after 16 hours of exposing in "Xenon-Arc-Fade-Ometer" | Percent decrease in max. density |
|------------------------------------------------------------------------------|----------------------------------------------|-----------------------------------------------------------------------|----------------------------------|
|                                                                              | 1.20                                         | 1.10                                                                  | 8.5                              |
|                                                                              | 1.20                                         | 1.03                                                                  | 14                               |
|                                                                              | 1.20                                         | 0.99                                                                  | 18                               |
| (color coupler for yellow according to British patent specification 808,276) |                                              |                                                                       |                                  |
|                                                                              | 1.20                                         | 0.84                                                                  | 30                               |
| (color coupler for yellow according to British patent specification 783,887) |                                              |                                                                       |                                  |

In connection with the structure of the color couplers according to the present invention, it is still to be noted that where the term "sulfonic acid group" or "sulfonic acid substituent" is used, the acid form as well as the salt form of this group or substituent is meant and the salt form preferably contains as cation and alkali metal cation, ammonium group or amine salt group.

We claim:

1. A photographic material comprising a silver halide emulsion layer and a color coupler for yellow which is a benzoylacetanilide coupler wherein the benzoyl part of the color coupler is directly substituted with at least one sulphonic acid group or substituted with a bivalent radical linked to a sulphonic acid-substituted phenyl group, and wherein the anilide part of the color coupler is directly substituted with at least one sulphonic acid group or substituted with a bivalent radical linked to a sulphonic acid-substituted phenyl group, said bivalent radical being a member of the group consisting of a —CONH— group, a —SO<sub>2</sub>NH— group, and a —NHCONH— group.

2. A photographic multi-layer color material containing in a non-migratory form in one of the light-sensitive silver halide emulsion layers or in a non-light sensitive water permeable colloidal layer adjacent to a light-sensitive silver halide emulsion layer, a color coupler for yellow which is a benzoylacetanilide coupler wherein the benzoyl part of the color coupler is directly substituted with at least one sulphonic acid group or substituted with a bivalent radical linked to a sulphonic acid-substituted phenyl group, and wherein the anilide part of the color coupler is directly substituted with at least one sulphonic acid group or

45 ing three silver halide emulsion layers optically different-  
ly sensitive including a layer selected from the group  
consisting of a blue sensitive silver halide emulsion layer  
and a non-light sensitive water permeable colloidal layer  
adjacent thereto, at least one of said layers containing a  
50 color coupler for yellow which is a benzoylacetanilide  
coupler wherein the benzoyl part of the color coupler is  
directly substituted with at least one sulphonic acid group  
or substituted with a bivalent radical linked to a sulphonic  
55 acid-substituted phenyl group, and wherein the anilide  
part of the color coupler is directly substituted with at  
least one sulphonic acid group or substituted with a bi-  
valent radical linked to a sulphonic acid-substituted phenyl  
group, said bivalent radical being a member of the group  
60 consisting of a —CONH— group, a —SO<sub>2</sub>NH— group,  
and a —NHCONH— group.

65 4. A photographic material comprising a silver halide emulsion layer and a color coupler for yellow having the general formula:



70 70 wherein

R<sub>1</sub> is a member selected from the group consisting of a sulphonic acid group and a salt thereof;  
R<sub>2</sub> is a member selected from the group consisting of a hydrogen atom and a sulfonic acid group, a salt form thereof, a halogen atom, and an organic group con-

taining an acyclic aliphatic radical with 5 to 20 carbon atoms in straight line making the molecule non-migratory;

$R_3$  is a member selected from the group consisting of a sulfonic acid group and a salt form thereof;  $R_4$  is a member selected from the group consisting of a hydrogen atom, and a sulfonic acid group, a salt form thereof, a halogen atom, and an organic group containing an acyclic aliphatic radical with 5 to 20 carbon atoms in straight line making the molecule non-migratory; and

$R_3$  and  $R_4$  together represent the necessary atoms for forming a sulfo-substituted aromatic system.

5. A photographic material comprising a silver halide emulsion layer and a color coupler for yellow having the general formula:



wherein

$R_2$  is a member selected from the group consisting of a hydrogen atom and a sulfonic acid group, a salt form thereof, a halogen atom, and an organic group containing an acyclic aliphatic radical with 5 to 20 carbon atoms in straight line making the molecule non-migratory;

$R_3$  is a member selected from the group consisting of a sulfonic acid group and a salt form thereof;

$R_4$  is a member selected from the group consisting of a hydrogen atom, and a sulfonic acid group, a salt form thereof, a halogen atom, and an organic group containing an acyclic aliphatic radical with 5 to 20 carbon atoms in straight line making the molecule non-migratory;

$R_3$  and  $R_4$  together represent the necessary atoms for forming a sulfo-substituted aromatic system;

$Y$  is a member selected from the group consisting of  $-\text{CONH}-$ ,  $-\text{SO}_2\text{NH}-$  and  $-\text{NHCONH}-$ ; and  $R'_1$  is a sulfonated aromatic radical.

6. A photographic material comprising a silver halide emulsion layer and a color coupler for yellow having the general formula:



wherein

$R_1$  is a member selected from the group consisting of a sulfonic acid group and a salt thereof;

$R_2$  is a member selected from the group consisting of a hydrogen atom and a sulfonic acid group, a salt form thereof, a halogen atom, and an organic group containing an acyclic aliphatic radical with 5 to 20 carbon atoms in straight line making the molecule non-migratory;

$R_4$  is a member selected from the group consisting of a hydrogen atom, and a sulfonic acid group, a salt

5  
10

form thereof, a halogen atom, and an organic group containing an acyclic aliphatic radical with 5 to 20 carbon atoms in straight line making the molecule non-migratory;

$Y_1$  is a member selected from the group consisting of a  $-\text{CONH}-$  group or a  $-\text{SO}_2\text{NH}-$  group; and  $R''_1$  is a sulfonated aromatic radical.

7. A photographic material comprising a silver halide emulsion layer and a color coupler for yellow having the general formula:



wherein

$R_2$  is a member selected from the group consisting of a hydrogen atom and a sulfonic acid group, a salt form thereof, a halogen atom, and an organic group containing an acyclic aliphatic radical with 5 to 20 carbon atoms in straight line making the molecule non-migratory;

$R_4$  is a member selected from the group consisting of a hydrogen atom, and a sulfonic acid group, a salt form thereof, a halogen atom, and an organic group containing an acyclic aliphatic radical with 5 to 20 carbon atoms in straight line making the molecule non-migratory;

$Y$  is a member selected from the group consisting of  $-\text{CONH}-$ ,  $-\text{SO}_2\text{NH}-$  and  $-\text{NHCONH}-$ ;

$R'_1$  is a sulfonated aromatic radical,

$Y_1$  is a member selected from the group consisting of a  $-\text{CONH}-$  group or a  $-\text{SO}_2\text{NH}-$  group; and  $R''_1$  is a sulfonated aromatic radical.

8. The photographic material of claim 1 wherein the color coupler is



40

45

50

55

60

#### References Cited

##### UNITED STATES PATENTS

|           |         |                   |         |
|-----------|---------|-------------------|---------|
| 3,112,198 | 11/1963 | Klinger           | 96-56.6 |
| 2,895,825 | 7/1959  | Pelz, et al.      | 96-56.6 |
| 2,950,314 | 8/1960  | De Cat, et al.    | 96-56.6 |
| 3,056,674 | 10/1962 | Hoffstadt, et al. | 96-100  |
| 2,662,913 | 12/1953 | Eberhart, et al.  | 260-507 |
| 2,836,620 | 5/1958  | Bersworth, et al. | 260-507 |
| 2,933,391 | 4/1960  | Feniak, et al.    | 96-100  |
| 2,983,608 | 5/1961  | Beavers           | 96-100  |

#### OTHER REFERENCES

Glakfides, "Photographic Chemistry," vol. 2, page 606, Fountain Press, London (1960).

J. TRAVIS BROWN, Primary Examiner.